

## UNITED STATES PATENT OFFICE

2,098,662

COPYING PAD AND METHOD OF PREPAR-  
ING SAMEWilliam Hoskins, Jr., La Grange, Ill., assignor to  
Ditto, Incorporated, Chicago, Ill., a corpora-  
tion of West VirginiaNo Drawing. Application May 23, 1936,  
Serial No. 81,513

15 Claims. (Cl. 41—31.6)

The present invention relates to improved hectograph copying pads or similar gelatinous copying pads and to methods of preparing the same.

Copy pads and bands of the hectograph type usually comprise a backing of paper, cloth or other suitable fabric and a coating or layer of some suitable gelatinous copying mass, which are bonded together by an intermediate layer or film formed from a drying oil such as linseed oil or the like. In the preparation of copying pads as hitherto carried out, the paper or fabric backing is first coated with a siccative oil such as linseed oil, tung oil, Perilla oil or the like, and the coating is then permitted to dry under normal atmospheric conditions until the coating hardens, forming a film or layer. This drying step usually takes from two to eight days. The prepared backing is then coated with a layer of some suitable gelatinous copying mass and the finished pad then shipped or stored for use.

This method is objectionable from the standpoint of the prolonged waiting time necessary to permit the intermediate siccative oil bonding layer to dry which necessitates the provision of large drying space and storage capacity; and because the bonding layer may in some cases harden unduly or fail to produce a bond of the required permanence.

In accordance with the present invention, I have found that the inherent disadvantages of the prior method of forming copying pads are overcome if a sulphonated oil product derived from a drying, semi-drying or non-drying oil is utilized as, or as a constituent of, the intermediate bonding layer between the backing and the copy mass. Not only does the sulphonated oil lend itself readily to quick drying by natural or artificial means, but the film formed is flexible and provides a permanent and effective bond between the backing and the gelatinous copy mass.

The copy mass embodied in the present invention may be suitably a gelatinous copying mass of the type frequently referred to as a hectographic copy mass; for example I may employ tanned gelatinous copying masses having suitable proportions of tanning agents, such as formaldehyde, alum or the like, or of light sensitive tanning agents such as the chromates or diox chromates; or I may use hardened gelatinous copy means, containing a glyceride of starch, as described and claimed in my prior co-pending application, Serial No. 48,495, filed November 6, 1935.

In carrying out the present invention, I may employ as the intermediate bonding layer a

water-soluble sulphonated oil, as for example sulphonated castor oil, sulphonated ricinoleic acid, Turkey red oil or the like. The sulphonated emulsifiable oil product may be applied directly or in solution to a sized cloth or paper or other suitable backing or I may incorporate the oil into a conventional sizing composition and apply it as such to the fabric backing to impregnate and coat the same.

Thus, I may employ for treating the fabric backing, an aqueous solution of a sizing composition containing suitably from about 3% upwardly of the sulphonated oil such as Turkey red oil or sulphonated castor oil. The proportion of sulphonated oil employed may be varied widely and may constitute as much as 25% to 50% of the size solution or even higher. As an example of a suitable size containing the sulphonated oil, the following, containing approximately 5% of sulphonated oil, has been found satisfactory:

|                     | Parts  |
|---------------------|--------|
| Glue.....           | 70     |
| Water.....          | 280    |
| Glycerin.....       | 445 25 |
| Turkey red oil..... | 40     |

The sizing composition containing the sulphonated oil is applied in any desirable manner to the paper, cloth or other suitable fabric backing and treated with a tanning agent to insolubilize the coating. If desired, suitable quantities of tanning agents, such as formaldehyde, aluminum alums or chrome alums may be employed in the mixture in proportions to secure some tanning action in the size.

The sized fabric backing containing the sulphonated oil is now quickly dried in any desirable manner, as for example by dry preheated air or gas, and is then coated with a layer of a gelatinous copying mass, suitably of the character above referred to. The drying may be rapidly effected as it is dependent upon various factors such as thickness of the sulphonated oil film, humidity, temperature of the heated air or other suitable heating means, etc. and not upon chemical, oxidizing or polymerization reactions as in the case of the bonding agents hitherto used. I have found that a backing treated in accordance with my invention may be suitably dried by heated air in about one-half hour. Obviously however, my invention is not dependent upon the exactitude of the time interval necessary to dry the sulphonated oil layer or film.

As set forth above, the sulphonated oil such as Turkey red oil, sulphonated castor oil or like

5 sulphonated drying, semi-drying or non-drying oil may be applied as such or in solution directly to a pre-sized backing and a layer of copy mass applied to the dried layer of oil. Thus, an aqueous solution of Turkey red oil containing 5% of the oil may be effectively used as the intermediate bonding layer. A 25% solution has been successfully used, and it is possible to utilize 50% solutions or even the sulphonated oil per se; however, these higher concentrations of the sulphonated oil are not necessary for the desired uniformly thin coating is more readily obtained at the lower concentrations.

10 The sulphonated oil product thus applied to 15 and forming a surface coating on the backing serves to effectively and permanently bond the surface copy mass layer to the backing.

15 If desired, the copy mass may be applied to the sized or coated backing while the latter is still 20 wet and the composite copy pad may then be set by cooling or in any desirable manner.

25 While I have described a preferred sizing composition containing the sulphonated oil, it is obvious that my invention is not to be construed as limited thereto, for the sulphonated oil may be used in conjunction with any conventional size either in admixture therewith or applied to a backing treated therewith.

30 In the specification, the expression copying pads is used to include pads in the form of long bands as used in rolls on copying machines as well as shorter pads and other forms of copying pads.

35 Although the present invention has been described in connection with the details of specific examples thereof, it is to be understood that it is not limited thereby except insofar as included in the accompanying claims.

I claim:

40 1. A copy pad comprising a backing, a copy mass and an intermediate bonding layer of a sulphonated oil.

45 2. A copy pad having a backing, a flexible bonding coating comprising a sulphonated oil on said backing and a layer of a copy mass on said coating.

50 3. A copy pad having a backing, a flexible bonding coating of a sulphonated oil on said backing and a layer of a gelatinous copy mass on said coating.

55 4. A copy pad having a backing and a gelatinous copy mass, the copy mass and the backing being bonded together by bond comprising Turkey red oil.

55 5. A copy pad having a backing and a gelatinous copy, the copy mass and the backing

being bonded together by a bond comprising sulphonated castor oil.

6. A copy pad comprising a backing, a gelatinous copy mass and an intermediate bond of Turkey red oil.

7. The method of preparing a copy pad which comprises applying to a backing a solution of a sulphonated oil to form a flexible bonding film, drying the film and applying a layer of a gelatinous copy mass to the treated backing.

8. The method of preparing a copy pad which comprises coating a sized backing with a solution of a sulphonated oil to form a flexible bonding layer, drying said layer and applying a layer of a copy mass to said bonding layer.

9. The method of preparing a copy pad which comprises coating a backing with a solution of Turkey red oil to form a flexible bonding layer and applying a layer of a gelatinous copy mass to said bonding layer.

10. The method of preparing a copy pad which comprises coating a sized backing with a solution of sulphonated castor oil to form a flexible bonding layer, drying said layer and applying a layer of a copy mass to said bonding layer.

11. The method of preparing a copy pad which comprises applying to a backing a size solution containing Turkey red oil to form a flexible bonding layer, drying said layer and applying a layer of a gelatinous copy mass to said bonding layer.

12. The method of preparing a copy pad which comprises applying to a backing a size solution containing Turkey red oil, a gelatinous sizing agent and a tanning agent to form a flexible bonding layer, drying said layer and applying a layer of a gelatinous copy mass to said bonding layer.

13. The method of preparing a copy pad which comprises coating a backing with a size solution containing at least 3% of Turkey red oil to form a flexible bonding layer, drying said layer and applying a layer of a gelatinous copy mass to said bonding layer.

14. The method of preparing a copy pad which comprises coating a backing with a solution containing about 5% of a sulphonated oil to form a flexible bonding layer, drying said layer and applying a layer of a gelatinous copy mass to said bonding layer.

15. The method of preparing a copy pad which comprises coating a backing with solution containing at least 3% of sulphonated oil to form a flexible bonding layer, drying said layer and applying a layer of a gelatinous copy mass to said bonding layer.

WILLIAM HOSKINS, JR.